

Patented Aug. 12, 1924.

1,504,338

# UNITED STATES PATENT OFFICE.

PIERRE GIRIN, OF PARIS, FRANCE, ASSIGNOR TO SOCIETE ANONYME DE COMMENTRY,  
FOURCHAMBAULT & DECAZEVILLE, OF PARIS, FRANCE.

## ALLOY COMPRISING IRON, NICKEL, CHROMIUM, TUNGSTEN, OR MOLYBDENUM.

No Drawing.

Application filed December 9, 1918. Serial No. 268,985.

To all whom it may concern:

Be it known that I, PIERRE GIRIN, a citizen of the Republic of France, residing in Paris, France, have invented certain new 5 and useful Improvements in a New Alloy Comprising Iron, Nickel, Chromium, Tungsten, or Molybdenum, of which the following is a specification.

The attainment of an industrial alloy having a high mechanical resistance at high 10 temperatures and capable of indefinitely preserving its properties, in spite of a prolonged exposure to these temperatures, is a problem which has not yet received a practical solution. In fact, the most resistant steels lose this property rapidly when their 15 temperature is raised from 400 to 500° C., and the hardness conferred by a suitable tempering disappears at the same time as the 20 reheating annuls the action of the treatment.

The "high speed" steels certainly preserve their hardness at a temperature higher than the other steels, and after they have 25 been tempered possess a high resistance, even up to a red heat, but besides the drawbacks which result from their fragility and difficulties of a practical nature due to the extremely high temperature of their treatment, they do not present the desired stability 30 when the temperature exceeds 600°; in fact, not only an accidental excess of temperature beyond the regulated value, but even prolonged exposure to this temperature produce a gradual disappearance of the initial 35 hardness and a progressive diminution of resistance. Finally, they are very oxidizable.

In addition, the invention of gas motors, 40 gas turbines and other thermal machines intended to act above the temperature of red heat, and the discovery of chemical synthetic processes using at the same time high temperatures and high pressures, render the realization of a metal possessing certain qualities at high temperature extremely desirable.

The present invention concerns an alloy of 45 iron, nickel, chromium and tungsten, and including, perhaps, molybdenum or vanadium, cobalt and titanium. This alloy is easy to obtain in large quantities, and capable of being moulded, forged, rolled, wire drawn, or otherwise worked, without difficulty, possessing at the temperature of 800° a resistance almost equivalent to that of cold 50 iron, non-fragile, practically inoxidizable at

high temperatures, even in a very oxidizing temperature, and at the same time possessing properties which are strictly reversible; by this term we understand that the properties at a given temperature depend solely on 60 that temperature and in no way on the preceding temperatures that have been obtained, nor on an exposure more or less long to the temperature used. The alloy may contain, for example:

|                             | Per cent.  |
|-----------------------------|------------|
| Nickel                      | 60 to 70   |
| Chromium                    | 10 to 15   |
| Tungsten                    | 2 to 5     |
| Manganese                   | 1 to 2     |
| Carbon                      | 0.3 to 0.6 |
| Iron forming the remainder. | 70         |

Certain variations in the composition may be admitted without introducing important modifications in the quality. We can replace the 2 to 5 per cent of tungsten by 1 to 3 per cent of molybdenum. The properties are still further improved and the manufacture facilitated by adding to the steel above defined 0.5 to 1 per cent of vanadium, or 80 0.1 to 0.2 per cent of titanium.

The alloy thus obtained forms a solid homogeneous solution; no thermal treatment can, consequently, modify its properties. The combined action of chromium and of 85 tungsten (this last metal being capable of being replaced wholly or partially by molybdenum) and, if it is present, of vanadium, is to confer on the alloy of iron and nickel a very high resistance when heated; we can obtain easily 25 to 35 kgs. per sq. mm. with an elastic limit of 20 to 30 kgs. and a coefficient of elongation of 40 per cent at a temperature of 800°, while still preserving a 90 total absence of fragility. These additional elements also render the alloy extremely resistant to the attack of acid vapours, as well as of hot oxidizing and moist gases. This chemical unalterability is of the greatest importance for all applications, since it not only ensures the metal against 95 corrosion, but also ensures the preservation of the initial mechanical properties, in contradistinction to that which takes place with carbon steels which, when heated for a long time in an atmosphere rich in hydrogen, finally become decarburized and lose their 100 solidity.

This alloy is certainly very suitable for 110 the manufacture of gas turbines, or for re-

ceptacles employed in chemical industry, for reactions which take place at high temperature and at high pressures, and which produce corrosive gases or other substances.

5 Having thus described the nature of the said invention and the best means I know of carrying the same into practical effect, I claim:-

A high nickel ferrous alloy containing 10 nickel, 60 to 70 per cent, chromium, 10 to 15 per cent, tungsten, 2 to 5 per cent, man-

ganese 1 to 2 per cent and carbon, 0.3 to 0.6 per cent, such alloy having at elevated temperatures great mechanical resistance and also great resistance to chemical agents and susceptible of retaining indefinitely its initial properties, notwithstanding prolonged service. 15

In witness whereof, I have hereunto signed my name.

PIERRE GIRIN.